

## UNITED STATES PATENT OFFICE

LESTER KIRSCHBRAUN, OF LEONIA, NEW JERSEY, ASSIGNOR TO THE FLINT KOTE COMPANY, OF BOSTON, MASSACHUSETTS, A CORPORATION OF MASSACHUSETTS

## PROCESS OF MAKING PAPER

No Drawing. Original application filed September 4, 1918, Serial No. 252,610. Divided and this application filed October 5, 1929. Serial No. 397,750.

This application is a divisional application of an original application filed by me September 4th, 1918, Serial No. 252,610.

This invention relates to a species of the 5 genus covered in my earlier application, Serial No. 252,607, filed September 4, 1918.

This invention relates to improvements in 10 process of making paper and has among its salient objects to provide a product which 15 while having the general characteristics of ordinary paper is distinguished therefrom by being waterproof; to provide a product which can be made upon commercial paper machinery; to provide a product in which 20 the waterproofing agent also acts as a continuous binder throughout the sheet; to provide a product which can be made with a much smaller percentage of fibre than is the case in ordinary paper and in which cheaper 25 fibres can be used but which at the same time makes a stronger and tougher product; to provide a product in which the waterproofing agent is incorporated in the body of the paper at the time the paper is formed; 30 to provide a novel and improved process of making the foregoing product and in which the stock containing the waterproofing agent will flow readily over the machine and will not stick thereto; to provide a process in 35 which the waterproofing agent as it passes with the fibres over the machine forms into a continuous body and which intermingles with the fibres and upon removal of the water coalesces, forming a unitary structure 40 with the fibre and in general to provide an improved process and product of the character referred to.

In the manufacture of paper attempts 45 have heretofore been made to saturate the finished product with a waterproofing agent. But difficulty has been experienced, particularly with certain kinds of fibre, in causing the waterproofing agent to thoroughly permeate throughout the paper. The operation 50 also is relatively expensive. Paper has, of course, been sized and the sizing incorporated with the stock before it passes over the machine. The present invention does not relate to either of the above processes.

55 Among the products for which the pres-

ent invention is adapted are paper provided with a design such as wall paper and ornamental paper. By the present invention these papers are made waterproof whereby that they can be readily washed when soiled, 55 without in any way deteriorating the paper. For example, wall paper made under the present invention, after it has been applied to the wall can be washed with soap and water. Other uses to which the invention 60 may be put are paper used for packing, for advertisements and generally paper subjected to the exposure of the weather. The product of this invention is also adapted for use for packing perishable articles or other 65 articles which might, for example, be subjected to moisture in storage or shipping. The product of this invention is also adapted for making containers which are not only 70 waterproof but germ proof and which can be cleaned and reused. In fact paper made in this way has a wide variety of uses.

The strength and flexibility of the paper 75 can be very largely controlled and varied within wide limits by the use of various kinds of binders and fibres. The paper can also be made of variable thicknesses and particularly relatively thin paper can be made in accordance with the present invention.

80 Not only can light colored paper be made by the present invention but paper of practically any color can be made, and a design of any desired configuration and color applied to the colored background or body of 85 the paper.

Describing now the process of the present invention, I make an aqueous paste, consisting of water and an emulsifying agent such as clay containing a substantial percentage of colloidal particles. In making 90 relatively white paper the clay should be white. Where colored paper is being made the color of the clay may be more or less disregarded. Other emulsifying agents 95 such as soap, starch dexterin and casein may be used and, if necessary, the emulsion produced with these agents, may be stabilized to the required degree. There are, of course, still other emulsifying agents than 100

those mentioned which may be suitable. This aqueous paste is preferably made with hot water, the water being heated to a temperature below 212° F., and in such cases I have found a temperature of 180° F., advantageous. In some cases I have found that equal parts of water and clay make a satisfactory paste.

To this paste is added the binder, preferably in a hot liquid condition. The binder may be gradually added to the paste while the latter is being stirred, hot water being added from time to time. This mixture is so stirred as to thoroughly amalgamate the paste and the binder; the object being to obtain a thorough dispersion of minute particles of the binder throughout the paste. The result is an emulsified matrix. This matrix is relatively non-sticky and can be thinned with water as desired. I have found, where clay is used, that five parts by weight of binder to one part by weight of clay makes a satisfactory matrix; although it is to be understood that the proportions may very widely vary, depending upon the characteristics of the product desired and the character of binder and the emulsifying agent.

With reference to the binder, it should of course be of a waterproof character and have a certain degree of adhesiveness. It also should have the ability to coalesce when the water is removed. When the color of the paper is of no importance black hydrocarbons such as natural and artificial asphalts, coal tar pitches and the like may be used. Animal and vegetable pitches may also be used. Where the body of the paper is to have a distinct color, such as red, green, blue or the like, the binder should be of a lighter hue, for example, resin or waxes softened with wax tailings, linseed oil or other oils may be used. In some cases the waxes might be used alone. The residue resulting from the redistillation of wax tailings may also be used. Whatever binder is used it is preferably mixed with a pigment of the desired color or with a dye soluble in the binder.

Where relatively white paper is desired the binder may consist of paraffin which may be treated to neutralize any yellowish shade in the usual manner.

This emulsified matrix is then intimately mixed with the fibre. Various kinds of fibres can be used. A few of them may be enumerated, such as wood pulp, rags, leather waste, linen, plant fibres and grasses. Instead of coloring the binder, the fibre may be colored. The mixture is now ready to be passed over the paper forming machinery. The machinery may be of a standard type such as a cylinder machine, or a Fourdrinier machine. If sheets of greater thickness are desired the stock may be run

over a board or "wet" machine. I have found that stock made in the way described will pass over a screen such as the screen of a Fourdrinier machine without sticking and will also pass over the felt belts or carriers without sticking. No difficulty will be experienced in drying the formed sheet. As the water dries out of the sheet the binder coalesces and forms a continuous waterproof structure throughout the sheet. The product will be much stronger and tougher than ordinary paper but can be made as flexible as desired.

If it is desired to put a design on the paper it may be printed on in the same way as designs are printed on ordinary paper. It is to be understood, however, that the ink or other material with which the design is applied should be of a waterproof character. Linseed oil may be used as the vehicle for the pigments used in the printing ink.

I claim as my invention:

1. A stock capable of being felted on a paper forming machine, consisting of a non-adhesive emulsion of water, colloidal clay, and a fusible waterproof light-colored base in which the water and clay form the external phase of the emulsion mixed with fibrous pulp.

2. A stock capable of being felted on a paper forming machine, consisting of a non-adhesive emulsion of water, an emulsifying agent, and a fusible waterproof light colored pitchy binder in which the water and emulsifying agent form the external phase of the emulsion, mixed with fibrous pulp, the binder at all times being chemically unaltered.

3. A non-adhesive emulsion of water, an emulsifying agent, and a fusible waterproof base, to which a coloring constituent has been added to impart a predetermined color in which the water and emulsifying agent form the external phase, mixed with a fibrous pulp, the stock so produced being capable of being felted on a paper forming machine.

4. A non-adhesive emulsion of water, an argilliferous emulsifying agent containing colloidal particles and a light colored fusible waterproof base, to which has been added a coloring constituent to impart a predetermined color thereto, in which the water and emulsifying agent form the external phase, mixed with fibrous pulp, the stock so produced being capable of being felted on paper forming machine.

5. A non-adhesive emulsion of water, an emulsifying agent and paraffin in which the water and emulsified agent constitute the external phase, mixed with fibrous pulp, the stock so produced being capable of being felted on a paper forming machine.

6. A non-adhesive emulsion of water, an

argilliferous emulsifying agent containing colloidal particles, and paraffin, in which the water and emulsifying agent constitute the external phase, mixed with fibrous pulp, the stock so produced being capable of being felted on a paper forming machine.

7. Fibrous stock capable of being felted on a paper making machine consisting of a non-adhesive emulsion of water, emulsifying agent and fusible waterproof, light colored base in which the water and emulsifying agent form the external phase of the emulsion, mixed with the fibrous pulp, the stock when sheeted resulting in a product in which the emulsion has been coalesced and constitutes a continuous waterproofing medium for the paper and being of light and non-odorous character whereby it has the capability 20 of use as containers for food products and the like.

Signed at Rutherford, in the county of Bergen and State of New Jersey, this 26th day of September A. D. 1929.

25 LESTER KIRSCHBRAUN.

30

35

40

45

50

55

60

65